

# UNITED STATES PATENT OFFICE.

FREDRIK W. DE JAHN, OF NEW YORK, N. Y., ASSIGNOR TO GENERAL CHEMICAL COMPANY, OF NEW YORK, N. Y., A CORPORATION OF NEW YORK.

## CATALYST FOR THE PRODUCTION OF AMMONIA AND PROCESS OF MAKING THE SAME.

1,159,365.

Specification of Letters Patent.

Patented Nov. 9, 1915.

No Drawing. Original application filed July 8, 1914, Serial No. 849,680. Divided and this application filed May 5, 1915. Serial No. 25,902.

To all whom it may concern:

Be it known that I, FREDRIK W. DE JAHN, a subject of the King of Norway, and a resident of the borough of Manhattan, city, 5 county, and State of New York, have invented certain new and useful Improvements in Catalysts for the Production of Ammonia and Processes of Making the Same, of which the following is a specification.

10 My invention relates to the synthetic production of ammonia and more particularly to a new catalytic agent therefor, its production and use.

15 The present application is a division of my application, which has become Patent 1,141,948, dated June 8, 1915.

I have discovered that if a gaseous mixture containing nitrogen and hydrogen is 20 suitably passed in contact with a suitable material composed essentially of (1) nitrogen, (2) an alkali metal such as sodium or potassium, and (3) one or more of the following metals, all of which are for the 25 pose of this invention equivalents:—manganese, cobalt, cerium, boron, titanium, uranium and silicon, the nitrogen and hydrogen of the gaseous mixture are united to form ammonia.

30 In order that my invention may be clearly understood, it is now set forth in the form of specific examples, it being understood, of course, that the invention is not to be limited to the exact materials or proportions thereof, 35 nor to the temperature or other conditions of the examples, since these may be varied without departing from my invention.

It is also to be understood that a catalyzer 40 may contain either manganese, cobalt, cerium, boron, titanium, uranium or silicon, together with an alkali metal and nitrogen, or may contain two or more of these metals together with an alkali metal and nitrogen; in the latter case the percentage of the 45 alkali metal plus nitrogen in the catalyzer is preferably not varied, that is to say, for example, if instead of cobalt in the catalyzer it is desired to substitute cobalt and titanium, the proportion of the cobalt and titanium combined, to the alkali metal and nitrogen combined, is substantially the same as the proportion of cobalt to the alkali metal and nitrogen combined, in the original cata-

lyzer, while the ratio of the cobalt to the titanium may be any ratio desired. In a 55 like manner, part or all of the particular alkali metal mentioned, say sodium, may be replaced by another alkali metal, as for instance, potassium. Moreover, the manganese, cobalt, cerium, boron, titanium, 60 uranium and silicon, whether said metals are used in the catalyzer singly or in associated relation, may be replaced in part by iron, nickel, and molybdenum, which last mentioned metals are more specifically referred 65 to and claimed in my Patent 1,141,947, dated June 8, 1915, the present invention being in the nature of an improvement over the invention of said patent.

Example I—Preparing the catalytic material.—Pumice stone in small pieces is purified by treatment with hydrochloric acid for about twenty-four (24) hours; it is then washed with distilled water until free from chlorid and then ignited to dryness.

A. Of this product 100 grams are treated with substantially the atomic weight in grams (59 grams) of cobalt in the form of nitrate dissolved in the necessary quantity of water, say 150 grams of water, and the whole is 80 evaporated to dryness, being stirred thoroughly during the evaporation; in this way the cobalt is to be uniformly distributed over the pumice. The thus treated pumice is now ignited at about 550° C. until fumes are 85 no longer given off and is then heated at about the same temperature in an atmosphere of hydrogen until water is no longer formed. To this product, when cooled in an indifferent atmosphere such as hydrogen and 90 while still in such atmosphere, add 69 grams of metallic sodium (or 117 grams of metallic potassium) in small pieces and then heat the whole for the purpose of melting the sodium and distribute the molten sodium 95 over the surface of the pumice material as, for example, by suitable continued stirring; displace the indifferent gas by anhydrous ammonia vapor or gas and heat the material to about 300° C. while passing ammonia vapor until a practically constant weight is obtained. Preserve the material, after being cooled, ready for use in, for example, a dry atmosphere of ammonia.

B. In place of the atomic weight in grams 105 of cobalt in the form of nitrate in the fore-

going Example A, I can use the atomic weight in grams of manganese or titanium, preferably in the form of chlorid.

C. In place of the hydrogen used in treating the ignited pumice and cobalt or the like material, I can use a mixture of nitrogen and hydrogen or other suitable reducing gas.

D. In the case of the elements cerium, uranium and silicon, I have found it advantageous to treat the prepared pumice with the chlorids of these elements in the same manner as with the nitrate of cobalt of the preceding and to effect the formation of a suitable product by the use of metallic sodium (in place of hydrogen) and heat; thereupon washing the result thoroughly with distilled water until water soluble chlorid has been substantially wholly removed; dry; then add metallic sodium as before and treat with anhydrous ammonia vapor or gas as before. For 100 parts of prepared pumice I treat: 140 grams of cerium in the form of chlorid with 69 grams of metallic sodium, or 28 grams of silicon in the form of chlorid with 92 grams of metallic sodium, or 238 grams of uranium in the form of chlorid with 92 grams of metallic sodium. (In place of the sodium I may use the equivalent amount of metallic potassium).

30 Heat the result of such treatment to about 300° C. until the further formation of sodium chlorid substantially ceases; then treat with hot distilled water until practically all the water-soluble chlorid has been removed; 35 now wash well with distilled water and dry by gentle heating in an indifferent atmosphere such as hydrogen; now add in each case 69 grams of metallic sodium or the equivalent amount of metallic potassium; heat 40 to a temperature just above the melting point of the sodium and distribute the molten sodium uniformly over the surface of the pumice material, as, for example, by suitable continued stirring. Now displace the 45 hydrogen or other indifferent gas by means of anhydrous ammonia vapor or gas and raise the temperature of the whole to 300° C. and maintain that condition until a practically constant weight is obtained; after 50 cooling preserve the material ready for use in a dry atmosphere of, for example, ammonia.

E. In the case of boron, I prefer to proceed as follows: I make a paste of the element in finely powdered condition (for example, in the so-called impalpable powder form) with water and thoroughly commingle this paste with the aforementioned prepared pumice while applying heat in sufficient and proper amount and rate to drive off substantially all of the water; add to the result a quantity of metallic sodium amounting to 69 grams of metallic sodium for each atomic weight in grams of the boron employed, which has been ascertained to have

been affixed to the prepared pumice in each case. Take the 69 grams of metallic sodium or their proportionate weight determined as above, in finely divided condition, and heat the whole in an indifferent atmosphere such as 70 hydrogen to just above the melting point of the sodium and distribute the molten sodium uniformly over the surface of the pumice material, as, for example, by continued stirring. Now displace the hydrogen or other indifferent gas by means of anhydrous ammonia vapor or gas and raise the temperature of the whole to 300° C. and maintain in that condition until a practically constant weight is obtained; after cooling preserve the material ready for use in, for example, a dry atmosphere of ammonia.

F. It is also useful to prepare catalysts containing more than one of the above named non-alkali elements. For instance, 85 in Example A, I can use in place of the 59 grams of the element cobalt, 29.5 grams thereof and 24 grams of the element titanium, both in the form of chlorid. I can use the 69 grams of sodium or a portion 90 thereof putting in the place of the omitted portion an equivalent amount of metallic potassium, or I may put in place of the 69 grams of metallic sodium 117 grams of metallic potassium.

In Example A, I can also use in place of the 59 grams of the element cobalt 16 grams each of the elements iron, cobalt and titanium, all in the form of chlorid. I can also suitably use combinations of the elements iron nickel and cobalt as mixed nitrates and chlorids as circumstances may indicate or make desirable.

The methods used in D or E above can also be applied to all the other elements if desired, but I prefer the methods above given for the respective elements recited. Sodium or potassium amid can be used and the pumice or other suitable carrier may be omitted.

By these methods or a suitable combination of all or part of them, it is possible to produce any desired combination of elements as catalysts.

*Example II—Utilizing the catalytic to produce ammonia.*—For producing ammonia about 175 grams of the product of Example A above, or a corresponding amount of its equivalent, are placed in a suitable catalytic chamber for ammonia synthesis and there is passed in contact with such catalyst a gas current preferably containing one volume of nitrogen for every three volumes of hydrogen. The gas mixture must be suitably purified and must be freed especially from contact poisons in the well known manner. With the pressure of the gas traversing the chamber within the range of 80 to 90 atmospheres and the temperature of treatment approximately be-

tween 520° C. and 540° C., I have succeeded in producing synthetic ammonia to the extent that the ammonia gas leaving the treating chamber constituted 4.5% by volume of the total gas leaving such chamber. The ammonia is removed from the gas discharged from the catalytic chamber in any suitable manner.

Wherever in this specification or in the claims annexed thereto I have used the word "cobalt", I mean, of course, to include therein each and all of the aforementioned equivalents thereof, either alone or in mixture with each other; likewise when in this specification or in the claims thereto annexed I have used the word "sodium", I mean to include in that term the equivalent thereof disclosed herein, namely, potassium. Moreover, when in the claims I specify broadly or specifically in the making of the catalyster that (A) cobalt (or its equivalent) is added to (B) an alkali metal, and the product thus formed is treated with (C) a gas containing nitrogen, I mean to include also the equivalents of such process, among which equivalents I mention the addition of (A) cobalt to the product resulting from the treatment of the metal (B) with the gas (C); the addition of the metal (B) to an oxid or suitable salt of the metal (A) followed by the reduction of the compound of the metal (A) as by hydrogen, the resulting product being then treated with the gas (C); and

the addition of a suitable compound, such as an amid, of the metal (B) to the metal (A). 35

I claim:

1. As a new article of manufacture, a substance containing cobalt, sodium and nitrogen, and which can cause nitrogen and hydrogen to combine to produce ammonia. 40

2. The herein described process of making a catalytic agent suitable for producing ammonia, which consists in adding (1) cobalt to (2) sodium and treating the product so formed with a basic gas containing nitrogen. 45

3. The herein described process of making a catalytic agent suitable for producing ammonia, which consists in adding (1) cobalt to (2) sodium and treating the product so formed with ammonia. 50

4. The herein described process of making a catalytic agent suitable for producing ammonia, which consists in treating a compound of cobalt with metallic sodium, removing water-soluble material from the product formed, then treating the result with metallic sodium and finally treating the resultant product with ammonia. 55

In testimony whereof I have hereunto set 60 my hand in the presence of two subscribing witnesses.

FREDRIK W. DE JAHN.

Witnesses:

JOHN A. FERGUSON,  
FRITZ ZIEGLER, Jr.